

# UNITED STATES PATENT OFFICE.

GEORGE FRANÇOIS JAUBERT, OF PARIS, FRANCE.

## PROCESS OF COMPRESSING PEROXID OF SODIUM.

SPECIFICATION forming part of Letters Patent No. 709,490, dated September 23, 1902.

Application filed April 23, 1901. Serial No. 57,115. (No specimens.)

*To all whom it may concern:*

Be it known that I, GEORGE FRANÇOIS JAUBERT, a citizen of the Republic of Switzerland, residing at Paris, France, have invented a new and useful Improvement in Processes of Compressing Peroxid of Sodium, of which the following is a specification.

My invention relates to the method of compressing peroxid of sodium into pastils or tablets.

The peroxid of sodium used in bleaching is only actually known in the form of a fine powder having a slightly-yellow appearance. When it is placed in contact with fabric or other inflammable material, the powder heats, as is well known, and even to such a degree as to fire the same. This powder of peroxid of sodium placed in water decomposes partially with brisk effervescence. It is therefore usually recommended to place the peroxids into the water slowly in small quantities only, at the same time constantly stirring in order to avoid a too-violent reaction, which may manifest itself as an explosion, by hissing, or boiling.

I have found that the peroxid of sodium which, as above stated, in the form of a fine powder or of very small perfectly-friable particles possesses, contrary to what would be expected from this last property, the property of agglomerating under strong pressure and without the aid of any agglutinant, giving to the compressed material very great hardness and very great density. Thus the density of ordinary peroxid of sodium in powder being about one, that of compressed peroxid of sodium will attain from 1.6 to 1.7. This compressed peroxid is very dense, very hard, and does not easily disintegrate. Placed in water, a slight disengagement of oxygen takes place at first, which soon ceases almost entirely, for it becomes covered at once with a layer of hydrate of peroxid of sodium, which dissolves slowly without giving rise to any tumultuous disengagement. This compressed peroxid of sodium, further, when placed in contact with inflammable substances is not dangerous in use, as is the powder of peroxid alone. By compression I avoid the two main objections to the peroxid of sodium—that is to say, its almost explosive decomposition in presence of water and the danger of fire. I

have also found that by agglomerating not only pure peroxid of sodium but a mixture in the proportions desired of peroxid of sodium and an acid salt—for example, bisulfate, polysulfate, and the like—or of a suitable dry organic or mineral acid there is obtained compressed material which placed in water and owing to the formation of neutral salts gives a solution of oxygenized water, either neutral, slightly acid, or slightly alkaline, according to the quantities of acid product in the compressed material.

I proceed in the following manner to obtain compressed peroxid of sodium. I usually make compressed pastils of five hundred grams or less and proceed as follows: I employ a steel pastil-mold of fifty-seven millimeters inside diameter and about two hundred millimeters high, formed of a cylinder closed at one end and in which a punch is forced by a powerful press giving seven thousand kilograms pressure upon the surface of the punch, whose area in this case is about twenty-five square centimeters. The cylinder being charged with five hundred grams of peroxid of sodium in powder, I cause the punch to descend, and after several blows of the press a cylinder of fifty-seven millimeters diameter and one hundred and twenty millimeters high may be taken out of the mold, it being absolutely hard and being of a density of from 1.6 to 1.7.

It is evident that with other molds or other pastil-machines may be made any size pastils desired by the consumer.

In order to compress the peroxid of sodium with the addition of bisulfate of potash, I proceed as in the above example; but instead of pure peroxid of sodium in powder I employ a very intimate mixture of thirty-nine parts of peroxid and of one hundred and thirty-six parts of bisulfate of potash melted and then pulverized. The mixture is compressed as above, and the pastil placed in water gives a neutral solution of oxygenized water. These pastils may be perfectly preserved in a stopped bottle.

I may replace the bisulfate by equivalent quantities of anhydrous bisulfate of sodium, anhydrous oxalic acid, tartaric acid, and the like or by a mixture of these acid products.

Having thus described the nature and ob-

jects of my invention, what I claim as new, and desire to secure by Letters Patent, is—

The method of compressing sodium peroxid, which consists in first pulverizing the sodium peroxid, then melting and pulverizing another salt, then mixing the pulverized sodium peroxid and the pulverized salt and finally compressing the mixture into pastils or tablets.

In testimony whereof I have signed this specification in the presence of two subscribing witnesses.

GEORGE FRANÇOIS JAUBERT.

Witnesses:

PAUL DE MESTRAL,

EDWARD P. MACLEAN.